

# United States Patent Office.

---

## IMPROVED ROOFING CEMENT.

---

SOLOMON B. MOORE, OF LOCKPORT, NEW YORK.

*Letters Patent No. 60,087, dated November 27, 1866.*

---

### SPECIFICATION.

TO ALL WHOM IT MAY CONCERN:

Be it known that I, SOLOMON B. MOORE, in the county of Niagara, in the State of New York, have invented a Cement or Composition for roofing purposes; and I do hereby declare that the following is a full and exact description thereof, and to the letters of reference marked thereon.

The nature of my invention consists in a combination of coal or gas tar, in proportions four to six quarts, mineral paint one quart, and pulverized lime-stone, (unburned,) made by sawing stone, (with an iron saw and sharp sand,) which will contain pulverized sharp sand and iron mixed with the stone-lime dust, (or the same ingredients produced in any other way,) sixteen quarts. These are mixed together in the proportions before stated, (or nearly so,) and spread with a trowel or brush upon felt paper, a sample of which is sent herewith, marked D. This composition is put on from one-fourth of an inch thick, to one-half of an inch thick, and will stand the water immediately, and hardens with age, so a person can walk upon the roof in three or four weeks.

What I claim as my invention, and desire to secure by Letters Patent, is—

The combination and using the materials as herein specified.

SOLOMON B. MOORE.

Witnesses:

G. W. HILDRETH,

JOSEPH CLARK.